

## 1

3,666,400

**SIZING OF YARNS AND FIBERS WITH COMBINATIONS OF POLYMERS AND CROSSLINKING AGENTS**

John T. Lofton and Robert J. Harper, Jr., Metairie, and Eugene J. Blanchard, New Orleans, La., assignors to the United States of America as represented by the Secretary of Agriculture

No Drawing. Continuation-in-part of application Ser. No. 756,323, Aug. 29, 1968. This application Mar. 10, 1970, Ser. No. 18,292

Int. Cl. D06m 13/52, 15/70

U.S. Cl. 8—115.6

5 Claims

**ABSTRACT OF THE DISCLOSURE**

This invention relates to a process for producing a durable-press fabric having a superior abrasion resistance. Cellulosic textile yarns are sized with a combination of a permanent polymer, a temporary polymer and a crosslinking agent prior to weaving. The permanent polymer includes polyurethanes, polyacrylates, butadiene-styrene copolymers, butadiene-acrylonitrile copolymers, and ethylene-vinylacetate copolymers. A temporary polymer is polyvinyl alcohol. Crosslinking agents include dimethylol dihydroxy-ethylenurea (DMDHEU), dimethylol methoxethylcarbamate, methylol melamine, and dimethylol propyleneurea.

This is a continuation-in-part of Ser. No. 756,323 filed Aug. 29, 1968, now abandoned.

A non-exclusive, irrevocable, royalty-free license in the invention herein described, throughout the world for all purposes of the United States Government, with the power to grant sublicenses for such purposes, is hereby granted to the Government of the United States of America.

The primary object of this invention is to provide a method for producing durable-press fabrics with superior abrasion resistance. In this method, textile fibers and crosslinking agents are sized with a combination of permanent polymer additive, temporary polymer agent and crosslinking agent prior to weaving. The polymer additive employed is one which improves the wrinkle recovery or abrasion resistance when applied to woven fabric. By application of the polymer additive to the yarn, prior to weaving, the polymer additive serves the dual purpose of acting as a weaving size and improving the wrinkle recovery of the finished fabric. The use of a crosslinking agent in conjunction with the temporary sizing agent provides a method by which the temporary agent becomes permanently attached to the fabric. By use of the crosslinking agent in the size, a less than normal amount of crosslinking agent can be utilized in finishing the fabric subsequent to weaving. This procedure provides a method of producing fabrics with smooth drying appearance and improved abrasion resistance.

Heretofore sizing mixtures have been designed to be temporary and are removed by desizing operations immediately after weaving. Permanent polymers are then applied to the fabric. Polymers applied to the fabric tend to stiffen the fabric and at times lead to undesirable yarn binding. This higher degree of stiffness is detrimental from the viewpoint of the esthetics of the fabric to the wearer as well as abrasion resistance in the garment manufactured from such fabrics.

By the process of this invention, polymers and crosslinking agents can be applied to yarns in the normal manner that starch size is applied. The types of polymers which have been successfully utilized have been polyurethanes, polyacrylates, and butadiene-styrene copolymers. The types of temporary sizing agents used in this research

## 2

include polyvinyl alcohol and carboxymethyl cellulose. The types of crosslinking agents used include dimethylol dihydroxyethylenurea and methylol melamines. The warp yarn is passed through the emulsion, squeezed, and dried and cured in some cases. The resulting warp beam is then loomed and woven into a fabric. The woven fabric can be scoured, bleached, and dyed. Durable-press crosslinking agents and other finishing auxiliaries are then padded onto the fabric and dried.

The advantages of using permanent polymer sizing are many. Polymers can be applied to the yarns in the normal manner that starch size is applied at the slasher. This eliminates the desizing procedure normally encountered in the application of a temporary sizing. Efficiency in weaving is equal to or better than regular starch size. It is also possible to vary the conditions of sizing. For example, you can use permanent sizing in warp and filling, permanent sizing in the warp direction only, or a combination of permanent and temporary sizing. Another advantage of applying the permanent polymer to the yarn and then weaving the fabric in contrast to application of the polymer to the woven fabric is that the resultant yarn treated fabrics are softer than the fabrics treated with the same polymer add-on. This reduced stiffness improves edge abrasion resistance. Durable-press fabrics, which have polymers only in the warp direction, do not have the exceedingly low crease sharpness values exhibited by fabrics which have been treated with the same polymers as fabric treatments.

Yarns can be sized with a combination of temporary and permanent sizing agents. This type formulation has cost advantages over the use of permanent sizing agents only. Under certain conditions temporary agents such as PVA/CMC can be crosslinked to produce fabrics with excellent durable-press performances and a substantial improvement in fabric strength properties.

In this method, textile fibers/yarns are sized with permanent polymers and combinations of these ingredients with crosslinking resins. This method produces good durable-press fabrics with low resin concentrations; thus improving physical properties with cost saving finishes. Directional application of polymer and crosslinking agents can be used to control physical properties, wrinkle recovery, and abrasion resistance of a preferred yarn direction in the finished fabric.

Other variations to this same basic treatment are also possible. A brief description and explanation of these variations will be given.

First, it is possible to prepare fabrics from polymer sized warp and filling yarns, and it is also possible to prepare fabrics from yarns treated with a combination of polymers and crosslinking agents. If the same polymer and crosslinking agent are used for both the warp and filling treatment, the resultant fabric is softer than the fabric treated with the same polymer. The yarn-treated fabrics then can be raised to durable-press performance with a lower level of crosslinking treatment or an equivalent level of crosslinking treatment. The yarn-treated fabric is softer and has improved abrasion resistance.

In a second variation, yarns were sized with one polymer in the warp direction and a second polymer in the filling direction. No such fabric can be produced from a fabric treatment and the types of polymers used for the warp and filling treatments can be used to control or modify final properties such as breaking strength, crease sharpness, fabric stiffness and other properties.

A special variation of sized warp and filling yarn fabrics can be employed to achieve certain unique fabric properties. Thus, it was found that heavyweight fabrics prepared from warp and filling polymer-treated yarns (particularly 2-ply yarns) can be used to produce a fabric

which has good wash-wear appearance with no further treatment other than application of a softener. Cuffs prepared from such fabrics showed good wash-wear appearance and crease sharpness through 30 launderings. The smooth drying and crease sharpness of such fabrics arise from the heat-set treatment of the polymer. Such fabrics, therefore, have the special advantage of no odor release in the cutting room. A second advantage would be that the fabric can be heat set later and as such an alterable garment can be produced by this method. A further refinement with these heavyweight goods is that the warp and filling polymer-treated heavyweight fabrics may be given a light crosslinking treatment, cured flat, washed, made into trousers and then heat set to produce crease and shape retention. This fabric has the same advantages as in the previous case (alterable pre-cure fabric, no formaldehyde odor in garment plants) with the further advantages of increased durable-press appearance and enhanced dimensional stability.

Another general area of variation in these yarn-treated fabrics would be to use a combination of permanent and temporary (standard) size in these yarn treatments. The temporary size may then be removed leaving the desired level of permanent size. This approach has the advantage of economy since the polymers used in permanent sizing generally are more expensive than temporary size agents. A further variation of the use of permanent and temporary sizing was observed when such fabric was crosslinked without any intermediate desizing operation. In several cases where both the warp and filling yarns were tested with combinations of permanent and temporary sizes and crosslinked without desizing, fabrics were obtained with 300° WRA and exceedingly high retention of breaking strength. For example, breaking strength retention was 96% in the warp direction and 85% in the filling direction. By contrast a conventional treatment on the non-polymer-treated (control) fabric had 39% retention in the warp direction and 32% retention in the filling direction.

Another general area of variation in these yarn-treated fabrics would be to use a combination of permanent and temporary size and crosslinking agents in the yarn treatments. Two variables are possible in this case. In one variation, a partial cure is applied to yarns so that only a part of temporary size is removed in the desizing operation. In the second case, a full cure is applied to yarns prior to desizing. By this latter method, most of the temporary size is converted to a permanent polymer additive on the fabric.

Permanent polymers which can be used by the process of this invention include polyurethanes, polyacrylates, butadiene-styrene copolymers, butadiene-acrylonitrile copolymers, and ethylene-vinylacetate copolymers in the range of about 4% to 20% by weight. With filling yarns, polymers can be used in the range from 1% to 20% and can also include silicones, polyethylene and polypropylene. Crosslinking agents include dimethylol dihydroxyethyleneurea (DMDHEU), dimethylol methoxyethylcarbamate, and methylol melamine propyleneurea in the range of about 1% to 20% by weight and temporary polymers include polyvinyl alcohol (PVA), carboxymethyl cellulose (CMC), and starch in the range of about 1% to 15% by weight.

The following examples illustrate but do not limit the scope of this invention. All percentages are by weight.

#### EXAMPLE 1

5 An 8-oz. twill fabric was woven from warp and filling yarns sized with 2% PVA and 2.7% low-temperature DMDHEU and 1% of a zinc nitrate base catalyst. Warp yarns were cured on slasher dry cans; filling yarns were cured in dye package form in dielectric heaters. In one case the fabric was boiled off, scoured and given a pad-dry cure using 3.6% DMDHEU and 1.4% of a zinc nitrate base catalyst. The second sample was given a pad-dry cure of 3.6% DMDHEU and 1.4% of a zinc nitrate base catalyst as it came from the loom. 10 A control fabric of untreated warp and filling yarn was desized, scoured, and given a pad-dry cure treatment using 6.3% solution of DMDHEU and 2.5% of a zinc nitrate based catalyst. All three fabrics had comparable wash-wear and crease ratings after the 1st and 20th wash cycle. Results are shown in Table I.

#### EXAMPLE 2

25 In another experiment the above fabric was woven from warp yarns treated with 2.5% solids polyurethane, 3% PVA, 2.7% solution DMDHEU and 1% of a zinc nitrate based catalyst, and an untreated filling. One portion of the fabric was desized, scoured, and treated with a 4% solution of DMDHEU. The other portion was 30 cured on a tenter frame at 320° F., desized, scoured, and treated with a 1.8% solution DMDHEU and 0.5% of a zinc nitrate base catalyst. Results in Table II.

#### EXAMPLE 3

35 In another experiment, a fabric was woven from warp yarns treated with 2.4% methylol melamine and 3% PVA and 0.5% of a zinc nitrate base catalyst. A partial cure was done on the steam cans and the fabric was then 40 scoured and repadded with 2.7% DMDHEU and 1% of a zinc nitrate base catalyst. The fabric was then dried and cured.

A second fabric was similarly treated except the warp finish contained 8% polyacrylate in addition to 3% PVA and 2.4% methylol melamine.

45 A control was also run in which the crosslinking agent was applied to the desized and scoured fabric only. The treatment consisted of 6.3% DMDHEU and 2.5% of a zinc nitrate base catalyst.

50 Results are shown in Table III.

#### EXAMPLE 4

55 In another experiment, the fabric was woven from warp yarn treated with 8% polyacrylate, 3% PVA, 1.4% DMDHEU and 0.5% of a zinc nitrate base catalyst. The filling yarns were untreated. After the fabric was woven, it was given a full cure. The fabric was then scoured and padded with 3.6% DMDHEU and 1.5% of a zinc nitrate base catalyst. The fabric was then dried.

60 A desized, scoured and bleached control twill fabric was padded with 8.1% DMDHEU and 3% of a zinc nitrate base catalyst. The fabric was dried and cured in the usual fashion. Results are shown in Table IV.

TABLE I

| Sample No. | Treatment                                                                                                                                                       | Flex abrasion |       | Grab strength |      | Tear strength |       | Wash-wear, 1st wash | Wash-wear, 20th wash | Crease, 1st wash | Crease, 20th wash |
|------------|-----------------------------------------------------------------------------------------------------------------------------------------------------------------|---------------|-------|---------------|------|---------------|-------|---------------------|----------------------|------------------|-------------------|
|            |                                                                                                                                                                 | Warp          | Fill  | Warp          | Fill | Warp          | Fill  |                     |                      |                  |                   |
| 5C7.....   | Control—6.3% sol. DMDHEU plus 2.5% of a zinc nitrate based solution. Desized-scoured.                                                                           | 57            | 118   | 49.7          | 54.7 | 1,367         | 1,433 | 5                   | 4.9                  | 5                | 4.9               |
| 5C5.....   | Warp and filling—2% PVA plus 2.7% DMDHEU (and 1% of zinc nitrate based solution) fabric—3.6% DMDHEU and 1.5% of a zinc nitrate based solution. Desized-scoured. | 178           | 467   | 62.5          | 66.5 | 1,650         | 1,700 | 4.7                 | 4.7                  | 4.8              | 4.6               |
| 5C9.....   | Warp and fill—2% PVA plus 2.7% DMDHEU and 1% of a zinc nitrate based solution. Loom run.                                                                        | 777           | 1,275 | 90.5          | 81   | 2,283         | 2,117 | 4.2                 | 4.1                  | 4.9              | 4.9               |

TABLE II

| Sample No.   | Treatment                                                                                                                               | Flex abrasion |       | Grab strength |      | Tear strength |       | Wash-wear, 1st wash | Wash-wear, 20th wash | Crease, 1st wash | Crease, 20th wash |
|--------------|-----------------------------------------------------------------------------------------------------------------------------------------|---------------|-------|---------------|------|---------------|-------|---------------------|----------------------|------------------|-------------------|
|              |                                                                                                                                         | Warp          | Fill  | Warp          | Fill | warp          | Fill  |                     |                      |                  |                   |
| 5C7-----     | Control—Desized-scoured, 6.3% DMDHEU and 2.5% zinc nitrate based catalyst.                                                              | 57            | 118   | 49.7          | 54.7 | 1,367         | 1,433 | 5                   | 4.9                  | 5                | 4.9               |
| 7-P-1-4----- | Warp—2.5% polyurethane, 3% PVA—2.7% sol. DMDHEU and 1% of zinc nitrate based catalyst, desized-scoured 1.8% sol. DMDHEU untreated fill. | 332           | 886   | 68.4          | 54.7 | 1,733         | 1,533 | 4.5                 | 4.7                  | 4.9              | 4.7               |
| 7-P-2-4----- | Cured 320° F., desized-scoured, 1.8% sol. DMDHEU and 0.5% zinc nitrate based catalyst.                                                  | 990           | 2,058 | 88.2          | 63.2 | 2,533         | 1,633 | 4.2                 | 3.5                  | 4.4              | 4.3               |

TABLE III  
[2 x 1 twill, 8.5 oz./sq. yd.]

| Sample No. | Treatment                                                                                                                              | Flex abrasion |         | Grab strength |         | Tear strength |         | CRA  |
|------------|----------------------------------------------------------------------------------------------------------------------------------------|---------------|---------|---------------|---------|---------------|---------|------|
|            |                                                                                                                                        | Warp          | Filling | Warp          | Filling | Warp          | Filling |      |
| 5C7-----   | Control—6.3% sol. DMDHEU plus 2.5% zinc nitrate solution. Desized-scoured.                                                             | 57            | 118     | 49.7          | 54.7    | 1,367         | 1,433   | 270  |
| 8P1-6----- | Scoured—2.7% sol. DMDHEU plus 1% of zinc nitrate based solution. Warp—3% PVA, 2.4% methylol melamine. Filling untreated.               | 13,008        | 13,337  | 1106          | 184     | 13,000        | 12,227  | 1243 |
| 9P1-6----- | Scoured—2.7% sol. DMDHEU plus 1% zinc nitrate based solution. Warp—8% polyacrylate, 3% PVA, 2.4% methylol melamine. Filling untreated. | 1,473         | 1,555   | 92            | 70      | 2,633         | 2,000   | 255  |

<sup>1</sup> Partial cure on cans.TABLE IV  
[2 x 2 twill, 8.5 oz./sq. yd.]

| Sample No. | Treatment                                                                                                                                                                          | Grab strength |         |      | Wash-wear | Crease |
|------------|------------------------------------------------------------------------------------------------------------------------------------------------------------------------------------|---------------|---------|------|-----------|--------|
|            |                                                                                                                                                                                    | Warp          | Filling | CRA  |           |        |
| 4C8-----   | Control—Desized, scoured, bleached. 8.1% sol. DMDHEU and 3% of a zinc nitrate based catalyst.                                                                                      | 65            | 53      | 281  | 4.7       | 5.0    |
| 15P8-----  | Warp—8% polyacrylate, 3% PVA, 1.4% sol. DMDHEU and 0.5% of a zinc nitrate based catalyst. Filling—untreated. Fabric—scoured—3.6% DMDHEU and 1.5% of a zinc nitrate based catalyst. | 187           | 168     | 1282 | 14.0      | 15.0   |

<sup>1</sup> Full cure before scouring.

We claim:

1. A process for producing a durable-press fabric with superior abrasion resistance comprising:
  - (a) treating cellulosic textile warp and filling yarns with an emulsion consisting of about from 4% to 20% by weight of a permanent polymer selected from the group consisting of polyurethanes, polyacrylates, butadiene-styrene copolymers, butadiene-acrylonitrile copolymers, and ethylene-vinylacetate copolymers, about from 1% to 20% by weight of a crosslinking agent selected from the group consisting of dimethylol dihydroxyethyleneurea, dimethylol methoxyethylcarbamate, dimethylol propyleneurea, and methylol melamine, and about from 0.5 to 1.5% by weight of a base catalyst, and drying and curing the thus-treated yarns;
  - (b) weaving a fabric from the treated, dried, and cured yarns of steps (a); and
  - (c) crosslinking the woven fabric from step (b) with about from 1% to 20% by weight of a crosslinking agent selected from the group consisting of methylol dihydroxyethyleneurea, dimethylol methoxyethylcarbamate, dimethylol propyleneurea, and methylol melamine.
2. A process for producing a durable-press fabric with superior abrasion resistance comprising:
  - (a) treating cellulosic textile warp and filling yarns with an emulsion consisting of about from 1% to 15% by weight of polyvinyl alcohol, about from 1% to 20% by weight of a crosslinking agent selected from the group consisting of dimethylol dihydroxyethyleneurea, dimethylol methoxyethylcarbamate, dimethylol propyleneurea, and methylol melamine, and about from 0.5% to 1.5% by weight of zinc nitrate base catalyst, and drying and curing the thus-treated yarns;
  - (b) weaving a fabric from the treated, dried, and cured warp yarns of step (a) and untreated filling yarns; and
  - (c) crosslinking the woven fabric from step (b) with about from 1% to 20% by weight of a crosslinking agent selected from the group consisting of dimethylol dihydroxyethyleneurea, dimethylol methoxyethylcarbamate, dimethylol propyleneurea, and methylol melamine.
3. A process for producing a durable-press fabric with superior abrasion resistance comprising:
  - (a) treating cellulosic textile warp yarns with an emulsion consisting of about from 4% to 20% by weight of a permanent polymer selected from the group consisting of polyurethanes, polyacrylates, butadiene-styrene copolymers, butadiene-acrylonitrile copolymers, and ethylene-vinyl acetate copolymers, about from 1% to 15% by weight of polyvinyl alcohol, about from 1% to 20% by weight of a crosslinking agent selected from the group consisting of dimethylol dihydroxyethyleneurea, dimethylol methoxyethylcarbamate, dimethylol propyleneurea, and methylol melamine, and about from 0.5% to 1.5% by weight of zinc nitrate base catalyst, and drying and curing the thus-treated yarns;
  - (b) weaving a fabric from the treated, dried, and cured warp yarns of step (a) and untreated filling yarns; and
  - (c) crosslinking the woven fabric from step (b) with about from 1% to 20% by weight of a crosslinking agent selected from the group consisting of dimethylol dihydroxyethyleneurea, dimethylol methoxyethylcarbamate, dimethylol propyleneurea, and methylol melamine.
4. A process for producing a durable-press fabric with superior abrasion resistance comprising:
  - (a) treating cellulosic textile warp yarns with an emulsion consisting of about from 4% to 20% by weight of a permanent polymer selected from the group consisting of polyurethanes, polyacrylates, butadiene-styrene copolymers, butadiene-acrylonitrile copolymers, and ethylene-vinyl acetate copolymers, about from 1% to 20% by weight of a crosslinking agent selected from the group consisting of dimethylol dihydroxyethyleneurea, dimethylol methoxyethylcarbamate, dimethylol propyleneurea, and methylol melamine.

agent selected from the group consisting of dimethylol dihydroxyethyleneurea, dimethylol methoxyethylcarbamate, dimethylol propyleneurea, and methylol melamine.

3. A process for producing a durable-press fabric with superior abrasion resistance comprising:

- (a) treating cellulosic textile warp yarns with an emulsion consisting of about from 4% to 20% by weight of a permanent polymer selected from the group consisting of polyurethanes, polyacrylates, butadiene-styrene copolymers, butadiene-acrylonitrile copolymers, and ethylene-vinyl acetate copolymers, about from 1% to 15% by weight of polyvinyl alcohol, about from 1% to 20% by weight of a crosslinking agent selected from the group consisting of dimethylol dihydroxyethyleneurea, dimethylol methoxyethylcarbamate, dimethylol propyleneurea, and methylol melamine, and about from 0.5% to 1.5% by weight of zinc nitrate base catalyst, and drying and curing the thus-treated yarns;
- (b) weaving a fabric from the treated, dried, and cured warp yarns of step (a) and untreated filling yarns; and
- (c) crosslinking the woven fabric from step (b) with about from 1% to 20% by weight of a crosslinking agent selected from the group consisting of dimethylol dihydroxyethyleneurea, dimethylol methoxyethylcarbamate, dimethylol propyleneurea, and methylol melamine.

4. A process for producing a durable-press fabric with superior abrasion resistance comprising:

- (a) treating cellulosic textile warp yarns with an emulsion consisting of about from 4% to 20% by weight of a permanent polymer selected from the group consisting of polyurethanes, polyacrylates, butadiene-styrene copolymers, butadiene-acrylonitrile copolymers, and ethylene-vinyl acetate copolymers, about from 1% to 20% by weight of a crosslinking agent selected from the group consisting of dimethylol dihydroxyethyleneurea, dimethylol methoxyethylcarbamate, dimethylol propyleneurea, and methylol melamine.

- mate, dimethylol propyleneurea, and methylol melamine, and about from 0.5% to 1.5% by weight of zinc nitrate base catalyst, and drying and curing the thus-treated yarns;
- (b) weaving a fabric from the treated, dried, and cured warp yarns of step (a) and untreated filling yarns; and
- (c) crosslinking the woven fabric from step (b) with about from 1% to 20% by weight of a crosslinking agent selected from the group consisting of dimethylol dihydroxyethyleneurea, dimethylol methoxyethylcarbamate, dimethylol propyleneurea and methylol melamine.
5. A process for producing a durable-press fabric with superior abrasion resistance comprising:
- (a) treating cellulosic textile warp yarns with an emulsion consisting of about from 1% to 15% by polyvinyl alcohol, about from 1% to 20% by weight of a crosslinking agent selected from the group consisting of dimethylol dihydroxyethyleneurea, dimethylol methoxyethylcarbamate, dimethylol propyleneurea, and methylol melamine, and about from 0.5% to 1.5% by weight of a base catalyst, and drying and curing the thus-treated yarns;
- (b) weaving a fabric from the treated, dried, and cured warp yarns of step (a) and untreated filling yarns; and

- (c) crosslinking the woven fabric from step (b) with about from 1% to 20% by weight of a crosslinking agent selected from the group consisting of dimethylol dihydroxyethyleneurea, dimethylol methoxyethylcarbamate, dimethylol propyleneurea, and methylol melamine.

## References Cited

## UNITED STATES PATENTS

|    |                                                       |         |               |             |
|----|-------------------------------------------------------|---------|---------------|-------------|
| 10 | 2,840,442                                             | 6/1958  | Abrams et al. | 117—139.5 X |
|    | 2,467,233                                             | 4/1949  | Rust          | 117—141 X   |
|    | 3,407,026                                             | 10/1968 | Mauldin       | 117—139.5 X |
| 15 | 2,859,189                                             | 11/1958 | Fallon et al. | 117—139.5 X |
|    | 3,321,819                                             | 5/1967  | Walter et al. | 117—139.5 X |
|    | 3,360,494                                             | 12/1967 | Bolinger      | 117—139.5 X |
|    | 3,350,162                                             | 10/1967 | Beck          | 117—139.5 X |
| 20 | WILLIAM D. MARTIN, Primary Examiner                   |         |               |             |
|    | T. G. DAVIS, Assistant Examiner                       |         |               |             |
| 25 | U.S. Cl. X.R.                                         |         |               |             |
|    | 8—116.3; 117—139.4, 139.5 A, 143 A 161 KP, UD, UC, UE |         |               |             |